

# UNITED STATES PATENT OFFICE.

ERNEST WYNDHAM MERRY, OF SHEFFIELD, ENGLAND, ASSIGNOR, BY MESNE ASSIGNMENTS, TO PYROTAN LEATHER CORPORATION, OF WILMINGTON, DELAWARE, A CORPORATION OF DELAWARE.

## TANNING HIDES AND SKINS.

1,427,221.

Specification of Letters Patent. Patented Aug. 29, 1922.

No Drawing. Application filed February 11, 1919, Serial No. 276,339. Renewed May 16, 1922. Serial No. 561,418.

To all whom it may concern:

Be it known that I, ERNEST WYNDHAM MERRY, a subject of Great Britain, residing at Sheffield, in the county of York, England, 5 have invented certain new and useful Improvements in Tanning Hides and Skins; and I do hereby declare the following to be a full, clear, and exact description of the invention, such as will enable others skilled 10 in the art to which it appertains to make and use the same.

This invention relates to the tanning of hides and skins and has among other objects the improvement of the method of tanning 15 with a solution of a soluble pyrophosphate and alum whereby a product of uniformly high quality is assured, and the process is maintained at a high standard efficiency.

Soluble pyrophosphates have been heretofore suggested as tanning agents in Letters Patent #1,039,150 and #1,191,527 wherein a process is described for the employment of a solution of pyrophosphate of sodium with alum and salt. The hides are subjected 20 to the action of such a solution after the usual preliminary cleansing and unhairing treatment, and under certain specified conditions, to deposit aluminum pyrophosphate in the interstices of the hide substance. The process described has attained 25 a wide commercial importance because of the high quality of the product, the inexpensiveness of the tanning agents and the relatively short time required to produce leather. The process described in said Letters Patent is particularly valuable in the production of fine white leathers. Colored leathers are also produced advantageously through the operation of the process, which in fact is universally applicable 30 to hides and skins of every character to produce leather of a uniform and distinctive quality.

I have discovered that the controlling 45 factor in the production of a satisfactory product in accordance with the teaching of the Letters Patent hereinbefore referred to is the careful control of the temperature. Relatively slight variations in the temperature employed, particularly an increase in 50 the temperature beyond a well defined maximum, results in deterioration in the quality of the product to a marked degree. The 55 product where the temperature rises materi-

ally above the maximum, hereinafter specified, lacks tensile strength, and becomes more or less brittle or "grain-cracky". By carefully limiting the temperature to a specified range, and particularly by positively preventing a rise in the temperature above a maximum I am enabled to produce leather of a uniform character and high quality from hides and skins of widely varying origin and texture. Success in the 60 commercial operation of the process of pyrophosphate tanning depends in fact upon such regulation of the temperature.

The range of temperature which I find to be best adapted for the practical operation 70 of the process lies between approximately 90° F. and 107° F., the latter temperature marking the danger point or extreme upper limit at which deterioration of the product commences, if the materials are permitted to 75 attain such a temperature for any considerable period. Preferably, the range of temperature is maintained between 95° F. and 105° F., the product resulting from the process, when carried out within this range, 80 being markedly superior and of uniform quality, regardless of the texture and weight of the hides or skins which are subjected to the tanning operation.

In carrying out the process, in accordance 85 with my invention, the hides are preferably subjected to the usual washing, liming, unhairing, and fleshing operations. The hides are then preferably bated and finally 90 washed in water or suitable cleaning solutions, until thoroughly clean and in suitable condition for the actual tanning operations. The details of the preliminary treatment may be widely varied and may follow 95 the established practice of tanyards or depart therefrom in various respects, the preliminary treatment forming no part of my present invention.

The thoroughly cleaned hides are then 100 subjected in a suitable receptacle, for example, a pit, drum, wheel, or paddle, to the action of the tanning solution which includes a suitable proportion of a soluble pyrophosphate, a soluble aluminum salt and a suitable material such as sodium chloride or common salt, for overcoming the astringent action of the aluminum salt upon the hide whereby it is maintained in porous condition to assimilate the active tanning 105 110

agents. Preferably, sodium pyrophosphate, ammonia alum, and common salt are employed although other available soluble pyrophosphates may be substituted, and any 5 soluble aluminum salt may be advantageously used. For example, soda alum, potash alum, aluminum sulphate, or aluminum chloride may be substituted for the ammonia alum.

10 The concentration of the solution with reference to the several salts may vary somewhat depending upon the particular character of the hide treated. Preferably, the relative quantity of the pyrophosphate to the 15 alum is maintained at the lowest ratio compatible with the successful accomplishment of the desired object. I have discovered that, depending upon the particular character of the hide treated, the ratio of pyrophosphate 20 to the alum may vary from 1:4 to 1:10, the higher proportions of pyrophosphate being desirable where the hides are heavy and close in texture, and the lower proportions being desirable in the treatment of skins and hides 25 of loose texture and relatively light weight. For general purposes, the range of relative proportions of pyrophosphate to alum may be limited so that the alum exceeds 5 but does not exceed 7 times the weight of the 30 pyrophosphate. In calculating the relative quantities of the respective ingredients, I refer to the crystallized alum containing 24 molecules of water of crystallization, and substantially chemically pure anhydrous 35 sodium pyrophosphate.

The hides are subjected in the receptacle, as hereinbefore stated to a suitable quantity of the solution, the water content of which may vary between 20 and 40 per cent of the 40 weight of the hide substance treated. The process is preferably carried out in a drum or wheel which permits a close regulation of the temperature and insures a thorough treatment of the hides by exposing every 45 portion thereof to the action of the solution. The initial temperature of the solution is governed by the necessity of dissolving the respective constituents and is in the neighborhood of 90° F. During the tanning operation the temperature tends to rise and, if the process is not carefully watched and the tendency governed by suitable control, it will eventually rise to a point considerably 50 above the maximum hereinbefore specified 55 with attending disastrous results to the product. In accordance with my invention the temperature is under control throughout the operation, a suitably arranged thermometer giving a continuous indication of the temperature. When the process is carried out in a wheel or drum the temperature may be reduced at intervals when necessary by stopping rotation of the wheel or drum and opening the door or closure thereof. The 60 65 contents of the drum or wheel thus remain

quiescent for a period sufficient to reduce the temperature as desired after which the process is continued with alternate exposure of the contents to reduce the temperature, as may be necessary to maintain it below the 70 maximum of 107° F. Preferably, as hereinbefore stated the temperature is never allowed to rise above 105° F., the best results being obtained when the range of temperature is between 95° F. and 105° F. 75

When the tanning operation is satisfactorily concluded the liquor is withdrawn and the hides are subjected to any of the usual finishing operations. If colored leather is to be produced the hides may be subjected to 80 the action of a solution containing a suitable coloring agent preferably containing a tannin.

My present invention is directed solely to the limitation of the temperature substantially throughout the tanning operation, whereby the rise in temperature above 107° F. is positively prevented. This I have found to result in the production of leather of uniform quality, regardless of the variation of other factors affecting the process. Such factors may be widely varied in applying the process to hides and skins of different quality and character to produce commercial leather, so long as the temperature is prevented from exceeding the maximum hereinbefore specified substantially 90 throughout the tanning operation. 95

Various changes may therefore be made in the ingredients, proportions, and method of 100 applying tanning agents to the hides or skins, so long as the temperature is maintained and prevented from exceeding the range as specified in the annexed claims.

I claim:

1. A method of tanning hides and skins which includes drumming the hides in a solution containing a soluble aluminum salt and a soluble pyrophosphate and stopping the drumming operation at intervals where by the temperature of the mass is limited not to exceed 107° F. 105

2. A method of tanning hides and skins which comprises subjecting them to the action of a solution including a soluble aluminum salt and a soluble pyrophosphate and intermittently cooling the mass thereby preventing the temperature thereof from exceeding 107° F. 115

3. A method of tanning hides and skins which comprises alternately subjecting the hides to agitation in contact with a solution including a soluble aluminum salt and a soluble pyrophosphate, and retaining them in a quiescent condition while still in contact with the solution until the temperature is reduced, and thereby preventing the temperature from exceeding 107° Fahrenheit. 120

In testimony whereof I affix my signature,  
ERNEST WYNDHAM MERRY,